

May 25, 1954

S. S. KISTLER

2,679,545

HIGH-TEMPERATURE RESISTOR AND METHOD OF OPERATING IT

Filed Sept. 15, 1950

2 Sheets-Sheet 1

Fig. 1



Fig. 3

Fig. 2

Inventor  
SAMUEL S. KISTLER

By George Gumpf  
Attorney

May 25, 1954

S. S. KISTLER

2,679,545

HIGH-TEMPERATURE RESISTOR AND METHOD OF OPERATING IT

Filed Sept. 15, 1950

2 Sheets-Sheet 2



Fig. 7



Fig. 4



Fig. 6



Fig. 5

SAMUEL S. KISTLER  
Inventor

By *George G. Gandy*  
Attorney

## UNITED STATES PATENT OFFICE

2,679,545

HIGH-TEMPERATURE RESISTOR AND  
METHOD OF OPERATING ITSamuel S. Kistler, West Boylston, Mass., assignor  
to Norton Company, Worcester, Mass., a corpora-  
tion of Massachusetts

Application September 15, 1950, Serial No. 184,926

14 Claims. (Cl. 13—20)

**1** The invention relates to high temperature electrical heating resistors.

One object of the invention is to provide an electric furnace capable of reaching high temperatures and of operating at high temperatures over a long period of time. Another object of the invention is to provide an electric furnace with an oxide resistor which will not channel. Another object of the invention is to provide a resistance element of such material, shape and characteristics that it can be operated at high temperatures without channeling and without burning out. Another object of the invention is to provide cold end portions for an oxide heating element.

Another object of the invention is to produce practical embodiments of oxide heating resistors. Another object of the invention is to provide heating resistors and furnaces utilizing them of particular utility in research laboratories for the attainment of high temperatures. Another object is to provide high temperature resistors that can be used in many different atmospheres. Another object is to provide a high temperature electric furnace for operation at temperatures above 1600° C. and even above 2000° C.

Other objects will be in part obvious or in part pointed out hereinafter. The invention accordingly consists in the features of construction, combinations of elements and arrangements of parts, as will be exemplified in the structure to be hereinafter described and the scope of the application of which will be indicated in the following claims.

In the accompanying drawings, illustrating two of many possible embodiments of the mechanical features of this invention:

Figure 1 is a vertical sectional view of a furnace having a resistor constructed in accordance with the invention.

Figure 2 is a vertical sectional view of another furnace having a resistor constructed in accordance with this invention to illustrate another embodiment.

Figure 3 is a plan view of the furnace of Figure 2.

Figure 4 is a graph illustrating stable and unstable conditions in such a furnace under different loads and at different temperatures.

Figure 5 is a graph of critical temperatures for a zirconia resistor in different ambient temperatures.

Figure 6 is a graph of the heat radiated per square centimeter of a zirconia resistor at the critical temperature for different ambient temperatures.

Figure 7 is an electrical diagram.

As conducive to a clearer understanding of certain features of the present invention it is pointed out that while it has long been known that

many oxides are electrical conductors at elevated temperatures, these oxides in general have negative temperature coefficients of resistance, especially those which seem from all standpoints to indicate usefulness as heating resistors. Since zirconium oxide, also referred to as zirconia, doesn't melt until the extremely high temperature of about 2700° C. is reached, it would at first blush appear to be an excellent material for a heating resistor; but besides having a negative temperature coefficient of resistance, it undergoes a sharp volume change upon heating and cooling. Also it is such a poor conductor at low temperatures that it must be heated by another

source of heat before it will operate. Hence when used as a heating resistor, the furnace has to be heated by another means in order to make the zirconia resistor or resistors conducting. Furthermore the negative temperature coefficient results in a decreasing resistance as the temperature rises and on a constant potential source the resistor either becomes progressively hotter and hotter until it burns out, or it cools off and ceases to conduct. Moreover the negative temperature coefficient of zirconia has caused rods made thereof to become molten along the axis because the current always tends to flow wherever the material is hottest. This phenomenon is known as channeling and has been pronounced in cases where furnaces have been provided with large oxide heating resistors. Channeling can also occur in tubular resistors, the material heating more along one side or axial strip, with consequent failure. Other difficulties have heretofore been encountered. One of the objects of this invention is to overcome such disadvantages and difficulties.

Referring now to Figure 1, a furnace constructed in accordance with the present invention may comprise a furnace body 10 made up of any suitable refractory material for example out of kaolin bricks. This furnace body 10 provides a chamber 11 in which the heat is developed by a zirconia resistor heating element 12 which as will be observed is in the form of a tube.

The zirconia tube 12 is made out of stabilized zirconia  $ZrO_2$  preferably stabilized with from 3% to 6% lime,  $CaO$ , and the material may be made in the following manner. An electric arc furnace of the type disclosed in U. S. Letters Patent No. 775,654 patented November 22, 1904 to Aldus C. Higgins is provided. Furnaces of this type comprising iron shells cooled all over with a cascade of water have been in use practically ever since the date of the above patent and are well known to electro-chemists and therefore need not be further described herein. A furnace mixture of zirconia ore, coke, iron, carbon, and lime ( $CaO$ ) is prepared. Various zirconia ores or partially purified zirconia powder can be used.

In general these are the zircon and baddeleyite ores. However chemically purified zirconia can equally well be used but is of course more expensive.

The quantity of carbon provided in the furnace mixture should be two-thirds of the theoretical quantity of carbon required completely to reduce the silica plus 100% of the theoretical quantity required to reduce all the other oxides (except the zirconia) to metal plus about 20% excess over all of these quantities. This quantity can be varied from the above with no excess to the above or with 40% excess. The reason why only two-thirds of the theoretical quantity of carbon required completely to reduce the silica is provided is that about one-third of the silica is volatilized during the furnacing operation. On the other hand the excess mentioned is provided because some of the coke is used up by combining with oxygen other than that provided by the oxides to be reduced.

The quantity of iron should be enough to form with the silicon that is reduced from silica a ferro-silicon having an iron content of from 75% to 85%. The purpose of the iron is to combine with the silicon to form a ferro-silicon alloy which has a much higher specific gravity than elementary silicon and therefore will go to the bottom of the furnace and, after solidification, form a ferro-silicon button containing also other reduction products that can readily be separated from the rest of the ingot. The amount of iron to add is enough to make with two-thirds of the silicon present in the ore a ferro-silicon having an iron content of from 75% to 85% minus the amount of iron obtained by the reduction of the iron oxide in the ore to iron and this of course must take into account that a small percentage of iron oxide remains in the final product.

The quantity of lime as a stabilizing agent to be added should be from 3% to 6% of the amount of  $ZrO_2$  in the ore. The reason for providing the stabilizing agent in the above percentages is that less will not satisfactorily stabilize the zirconia, and more will form a eutectic thus making the product less refractory. The stabilizing agent in the range given causes the zirconia to crystallize predominantly in the cubic system, but when less of the stabilizing agent is used the crystals are predominantly monoclinic. Ordinary or natural baddeleyite is monoclinic whereas the product of this invention is predominantly cubic. The monoclinic form of zirconia will not withstand many cycles of heating to over  $2000^\circ C$ . and cooling to  $100^\circ C$ . and even lesser temperature changes may cause cracking or fracturing of the heating element if it is made of monoclinic zirconia. A zirconia of predominantly cubic crystal form will, however, withstand heat shock for many cycles. When the lime is as much as 6% the crystals are nearly all cubic, when the lime is as low as 2.7% about 35% of the crystals are cubic. Zirconia having 3% to 6% of lime on the  $ZrO_2$  is referred to as stabilized zirconia; the expression "stabilized" means that the zirconia does not have a detrimental volume change at the critical temperature of inversion of baddeleyite, normally about  $1000^\circ C$ . However I do not want to be limited to lime stabilized zirconia nor to the precise furnace operation described herein since magnesium oxide (3% to 6%) is likewise a stabilizing agent and other processes of combining the stabilizing agent with the zirconia can be effectively used. However the best material now known to me for

the manufacture of the resistor heating elements 12 is that above described.

For the manufacture of tubes of zirconia I may take zirconia grain and slip cast it, ram it, or 5 extrude it to form the "green" shapes, then dry the shapes and fire them at cone 35. However a very convenient way is to press the material to produce the tube shapes. The grit size of the zirconia has some relation to the size of the tube, 10 for example it is not desirable to try to make very small tubes with coarse grit. However this matter is not critical and the ceramist will readily know how to select proper grit sizes especially in view of the following example:

15 For the manufacture of a stabilized zirconia tube 6 inches long with a  $1\frac{1}{2}$  inch diameter bore and a  $1\frac{3}{4}$  inch outside diameter, I selected stabilized zirconia of grit sizes 24 mesh and finer down to 2 microns. This was simply the material produced by grinding the zirconia until it 20 would pass a 24 mesh screen. This grain was wet with a solution of 2% water and 1% dextrose, the percentages being on the weight of the zirconia. This wet mixture was then charged 25 into a rubber mold having a steel arbor and was pressed at 5000 pounds to the square inch. The molded "green" tube was then stripped from the mold, was dried and was fired at cone 35. This tube containing about 5% of lime on the total  $ZrO_2$  made a highly satisfactory heating resistor.

30 Referring again to Figure 1, the resistor 12 is seated in intermediate cold ends 13 which are likewise made of stabilized zirconia and can be fashioned out of the material above described 35 in the manner above described but steel molds can be used as it is not necessary to use a rubber mold to make cylindrical blocks such as the cold ends 13. These cold ends 13 have approximately four times the cross section of the tube 12 and consequently should have one-fourth the resistivity of the tube 12 at the same temperature. Within the scope of my invention the cold ends 40 13 should have at least twice the cross section of the tube 12 and I cannot give an upper limit because the greater the cross section of the cold ends 13 the better will be the performance of the furnace, only there are of course practical limitations on indefinitely increasing the size of these cold ends.

45 In contact with the intermediate cold ends 13 are outer cold ends 14 made of material which at practically any temperature has a lower resistivity than that of zirconium oxide, stabilized or otherwise. These outer cold ends 14 may, as shown, be cylindrical blocks and preferably they have nicely ground plane surfaces 15 in contact with equally nicely ground plane surfaces 16 on the ends of the cold ends 13. These outer cold ends 14 may be made of any oxide selected from the group consisting of zinc oxide  $ZnO$ , titanium oxide  $Ti_2O_3$ , magnetic iron oxide  $Fe_2O_4$ , copper oxide  $Cu_2O$ , manganese oxide  $Mn_3O_4$ , and uranium oxide  $UO_2$ . However from all standpoints including especially cost, I prefer zinc oxide,  $ZnO$ .

50 It is preferable that the oxide used be not very pure. The listed oxides are all of them more conducting if some impurities are present since defects in the crystal lattice, promoted by strain from foreign atoms or a deficiency or excess of 55 one of the atoms of the oxide, considerably increase the conductivity. Mixtures of any two or more of these oxides mentioned can be used and reduced products are certainly not excluded, but on the other hand are desirable and foreign material of almost any kind is not detrimental and

naturally any free metals present increase the conductivity. It is therefore not possible to give limits on the purity of the material of the outer cold ends 14 since clearly if copper oxide contained so much free copper present that there was only 1% of  $Cu_2O$ , it would be more conductive than pure  $Cu_2O$ . But on the other hand the purpose of using an oxide at all for the outer cold ends would be defeated by using almost pure metal so therefore the only definition I can give is the melting point of the material. The melting point of the outer cold ends should be no lower than  $1200^{\circ}C$ . The following table giving the melting points of metals and oxides may be helpful in this connection.

TABLE  
Melting points of metals and oxides

| Metals    | ° C.   | Oxides    | ° C.    |
|-----------|--------|-----------|---------|
| Zinc      | 420    | ZnO       | 1,900   |
| Copper    | 1,083  | $Cu_2O$   | 1,235   |
| Iron      | 1,535  | $Fe_3O_4$ | d 1,538 |
| Manganese | 1,260  | $Mn_3O_4$ | 2,705   |
| Titanium  | 1,806  | $Ti_2O_3$ | 2,130   |
| Uranium   | <1,850 | $UO_2$    | 2,176   |

d=decomposes.

As a specific example of the composition for the outer cold ends 14 I took a quantity of granular zinc oxide  $ZnO$ , technical grade, mixed it with water and dextrene to make a moldable material, pressed it into blocks and calcined them at  $1300^{\circ}C$ . for two hours. I then crushed these blocks to granular material 20 mesh grit size and finer. I then took 60% of the material so made and 40% of the original lot of granular zinc oxide, technical grade, mixed thoroughly, added 2% of dextrene and 2½% of water, mixed thoroughly again, placed this mix in molds of the desired size and shape, pressed pieces from this latter mix at 3000 pounds per square inch, stripped the pieces from the molds, dried them and fired them to  $1300^{\circ}C$ .

Referring again to Figure 1, the outer cold ends 14 should be resiliently pressed against the intermediate cold ends 13 and this can be done in any manner. As shown the furnace body 10 rests upon a steel plate 17 and to this steel plate 17 are fastened L-shaped springs 18 by means of screws 19 extending through slots 20 in the ends of insulating plates 21, the screws 19 being beyond the sides of the horizontal portions of the springs 18 so that the springs 18 are insulated from the plate 17. The upper ends of the springs 18 contact the outer ends of leads 22 that extend into the cold ends 14 as shown and have a snug fit therein. These leads 22 are preferably made of a nickel iron chromium alloy such as

60Ni24Fe16Cr

with .1 to .7 carbon.

It will be seen that the outer cold ends 14 are entirely outside of the furnace body 10 although they may be located in recesses 23 therein as shown. They are heated, of course, by conduction and so therefore have to withstand high temperatures but since they are located in the free air of the room where the furnace is located they will never rise to such high temperatures as will the intermediate ends 13. Consequently even though the heating element 12 may be as hot as  $2600^{\circ}C$ . the outer cold ends 14 will not melt even though they have a melting point as low as  $1200^{\circ}C$ .

The chamber 11 of the furnace may have any

desired shape but for convenience in constructing it as well as in using it, it may have a rectangular parallelepipedal shape. At least on one side of the chamber 11 and preferably on each side thereof is a removable brick 25 for gaining access to the chamber 11 and for admitting a flame thereto and exhaust gases therefrom in order to start the furnace in operation.

Electric current can be conveyed to the leads 22 via the springs 18 by means of copper conductors 27 connected to the springs 18 by binding posts 28 having nuts 29.

Figure 2 illustrates another embodiment of the invention in which the zirconia resistor heating element 32 also functions as a furnace wall. In this embodiment there are intermediate cold ends 33 which have an annular shape and these are in contact with outer cold ends 34 also having an annular shape. The outer cold ends 34 have nicely ground plane surfaces 35 in contact with equally nicely ground plane surfaces 36 on the intermediate cold ends 33. The lower cold end 34 rests upon a batt 37 of ceramic bonded silicon carbide or other insulating and refractory material. Just above the batt 37 is an annular plate 39 which may be made of sintered alumina. Inserted into and extending radially from the outer cold ends between the batt 37 and the annular plate 39 are a plurality of leads 42 which may be made of the same nickel iron chromium alloy as above described and similar leads 42 are imbedded in and extend radially from the upper outer cold end 34.

Just outside of the heating element 32 and resting upon the lower intermediate cold end 33 is a heat retaining zirconia tube 43, preferably made of the same stabilized zirconium oxide as already described. Resting upon the annular plate 39 and extending upwardly concentric with the tube 43 and the heating element 32 is a cylindrical steel shell 44. Between the steel shell 44 and the zirconia tube 43 is packed a quantity of zirconia grain 45 which may be of the stabilized variety or otherwise. Resting on this grain 45 and surrounding the upper intermediate cold end 33 is a short tube 46 made of sintered alumina. This furnace may have a hearth block 47 located inside of the lower cold ends 33 and 34, this hearth block 47 being preferably made of the aforesaid stabilized zirconia. Resting on the upper outer cold end 34 and extending well into the bores in this cold end and the cold end 33 below it is a furnace cap 48 likewise preferably made of the same stabilized zirconia. This cap 48 has a sight hole 49.

The annular plate of alumina 39 rests upon a steel ring 50 having radial holes through which extend the leads 42. There is another ring 50 at the top of the furnace which is clearly illustrated in the plan view of Figure 3. Strip metal springs 52 are secured by screws 53 to the top ring 50 and also to the bottom ring 50 and the ends of the springs 52 engage the outer ends of the leads 42 thus causing the latter to exert pressure against the cold ends 34 in which they are imbedded, for the purpose of making good electrical contacts. Electric current can be conveyed to the rings 50 and thence to the leads 42 by means of conductors 55 attached to the rings 50 by screws 56. In Figure 3 a cable 57 is shown connected to the conductor 55 and, of course, there is a similar cable (not shown) connected to a similar conductor attached to the lower ring 50.

Illustratively, the dimensions of the tube 32 of Figure 2 may be a length of 6 inches, an inside

diameter of  $3\frac{1}{8}$  inches, and an outside diameter of  $1\frac{3}{4}$  inches. It may be constructed in the manner above described in connection with the making of tube 12 of Figure 1, illustrative dimensions for which I have also given above. These dimensional relations between diameter and wall thicknesses are predetermined according to my invention so that the wall thickness of the zirconia tube is not too thick relative to the diameter of the tube and meets the criterion that

$$\frac{ID}{Wa} \text{ is not less than } 2$$

where ID is the inside diameter of the tube and Wa is the wall thickness. This preferred aspect of my invention will presently be further amplified. It is a factor that contributes toward overcoming limitations and difficulties heretofore encountered and toward achieving a number of practical advantages and results heretofore impossible so far as I am aware.

As above indicated, the end faces or surfaces of the tubular element 12 of Figure 1 and of the tubular element 32 of Figure 2 are preferably shaped or faced, as by grinding, to give even and uniform surface contact with the intermediate blocks or cold ends 13, 13 in Figure 1 and 33, 33 in Figure 2, and the latter may also be similarly faced or treated on those portions where they engage the resistor tube, thus to aid in achieving uniform contact resistance throughout the engaged surfaces whereby substantial uniformity of current flow per unit area of the cross-section of the resistor tube is more nearly achieved. Each resistor tube, being a hollow cylinder, may be regarded as comprising a number of individual longitudinal resistor elements arranged in a circle and in intimate side wall contact with each other and each carrying the same amount of heating current therethrough, and if the resistor tubes are dimensionally within the above criterion, it is possible to achieve operation of the resistor and of the furnace without materially disturbing the just described uniformity of current flow through these imaginary longitudinal subdivisions or elements of the hollow cylinder, as will be later described.

Uniformity of the surface contacts just mentioned above and also of the surface contacts between the intermediate cold ends and the outer cold ends whose contacting faces are also preferably ground, as above noted, is further enhanced by the continuity of the yielding pressures with which these serially successive surfaces in each of the illustrative furnace constructions are held in engagement with each other. In the construction of Figure 1 the spring arms 18, 18 supply and maintain this contact pressure, and in the construction of Figure 2 it is the weight of the successively stacked parts that furnishes this continuous but yielding pressure. Moreover the feature of yieldability also permits the various pressed-together parts to partake of dimensional changes in response to temperature changes, all without subjecting any of the parts to detrimental stress and without disturbing the uniformity and continuity of application of the contact pressure.

The furnace may be energized from any suitable source of current, preferably an alternating current source, as is diagrammatically indicated in Figure 7, and to the output thereof the furnace of Figure 1 or the furnace of Figure 2 may be connected through a suitable switch (not shown). The electrical system comprises any

suitable means for automatically maintaining constancy of current supply thereto and for purposes of illustration I have indicated in Figure 7 any suitable form of constant current regulator, preferably one in which the standard or magnitude of the current value to be kept constant may be manually set.

As previously stated, the furnace of Figure 1 can be started by a gas flame introduced through the hole which is left when a brick 25 is removed, the exhaust gases emerging through the hole on the other side, the other brick 25 being also removed. I have found that it is sufficient to heat the element 12 to about  $1400^{\circ}$  C. to start the furnace as after that the element 12 will carry enough current to continue the heating and raise the temperature gradually to that desired. The furnace of Figure 2 can conveniently be started by removing the hearth block 41 and the cap 48, placing a silicon carbide resistor vertically through the entire furnace (the batt 37 having a hole 59 in the bottom, as shown), energizing the silicon carbide resistor, thus heating the element 32 to about  $1400^{\circ}$  C., then removing the silicon carbide heating element, replacing the hearth block 41 and the cap 48, and turning on the current through the element 32.

According to my invention, I am enabled to achieve such substantial freedom from hazards and deficiencies heretofore met with as to make possible the reliable operation of oxide heating elements of large surface area. In operating the furnace, according to my invention, the initial heating of the tube element is effected in a manner to avoid giving rise to ruinous conditions of instability and, once it is heated and the electric current applied, I again effect controls and conditions that avoid instability, and in these connections the dimensional criterion of the tubular heater element plays a part.

If a constant potential is applied to the resistor and the furnace is heated by some means, such as a gas burner, until the resistor becomes conducting, the conditions are in general unstable and, without more, the temperature will increase until the element is destroyed. On the other hand, if the applied voltage is so controlled that the temperature does not run away, the likelihood is that one side of the tube will become warmer than other parts, thus becoming a better conductor leading to a heavier current therethrough which in turn leads to still higher temperature until virtually all of the current is channeling down one side of the tube which usually results in breakage. It is this sort of thing that has been one of a number of major factors heretofore limiting the uses of conductive oxides and preventing employment in heating elements of large surface area.

According to my invention, these obstacles are overcome. I have investigated the factors involved therein and as of aid in describing how I overcome the above obstacles, let it first be assumed that an element, sufficiently small in diameter to heat uniformly throughout the cross section (say, on the order of 2 millimeters), is enclosed in a furnace maintained at a constant temperature  $T_0$ . If a small current is passed through the element, heating it to some temperature  $T$  above that of the furnace, it will lose heat to the furnace through convection and radiation. At least, as a first approximation, one can reasonably represent the heat loss by the equation

$$H = k(T - T_0) \div k'(T^4 - T_0^4) \quad (1)$$

in which  $H$  represents the heat lost per square centimeter in watts,  $k$  is the heat transfer coefficient through convection, and  $k'$  is the heat transfer coefficient through radiation. Temperatures are on the Kelvin scale. As a first approximation, I have taken the values of  $k$  and  $k'$  as  $2 \times 10^{-2}$  and  $1.75 \times 10^{-12}$  watts. For practical purposes, at temperatures of interest in this art, the first term in the equation can be neglected. In calculating  $k'$  it was assumed that the emissivity of zirconia is 30% of black body. This figure is based upon measurements made in a laboratory.

Accordingly the heat lost from the heating element at any temperature above the furnace temperature can now be calculated. Knowing the resistance of zirconia at any temperature, the E. M. F. required to supply the heat lost can be calculated. Such calculations have been made for a tube of large bore with a wall thickness of 2 millimeters (in effect representing a series of small-cross-sectional elements arranged in a circle), and the results are plotted in Figure 4 for two furnace temperatures,  $1000^{\circ}$  K. (abscissae at the top) and  $1600^{\circ}$  K. (abscissae at the bottom). It is assumed, for the moment and for purposes of this analysis, that this very thin tube remains at uniform temperature throughout its cross section.

The specific resistance of lime-stabilized zirconia has been measured over a wide temperature range, and while there are variations due to impurities, porosity, and grain size distribution, it can be represented reasonably well by the equation

$$\log_{10} R = \frac{5960}{T} - 2.82 \quad (2)$$

Both curves of Figure 4 go through a definite maximum, although the one for  $T_0 = 1000^{\circ}$  K. rises much more steeply and attains its maximum much sooner than the other. At any temperature and constant voltage to the left of the maximum point the element will be stable, any fluctuation causing a higher temperature resulting in more energy being radiated than is generated, and the temperature will fall back to the equilibrium position. On the other hand, any potential and temperature to the right of the maximum point will lead to eventual run-away conditions, since any accidental displacement of the temperature upwards will cause a greater generation of heat than can be radiated and the temperature will rise at a progressively faster rate until fusion occurs.

Furthermore, the element is permanently unstable at any voltage above the maximum point. In this connection it should be pointed out that the voltage at the maximum point decreases as  $T_0$  is increased, so that a potential that is safe at a low furnace temperature may become excessive as the furnace heats up.

The relation between the critical temperature (i. e., the temperature at maximum voltage) and the furnace temperature is given in Figure 5 and the following equation

$$T^4 - \frac{4}{B} T^5 = T_0^5 \quad (3)$$

In this equation,  $B$  comes from the variant of Equation 2

$$R = A e^{B/T} \quad (4)$$

in which, for stabilized zirconia,  $A = 0.00152$ , and  $B = 13,700$ . Note that  $A$ , which contains such factors as porosity, grain size, shape

of cross section of the element, and magnitude of the specific resistance, does not appear in Equation 3. It is inconsequential, therefore, from a stability standpoint, how the heating element is formed as long as the activation energy of the conduction process is not affected.

Figure 5 shows that at low temperatures the critical temperature is very little above the ambient temperature, thus providing only a narrow region of stability, while at high furnace temperatures the stability limits are very wide. At furnace temperatures above  $1800^{\circ}$  K., instability is no longer possible with a voltage below that necessary to melt the zirconia element.

In Figure 6 is plotted the heat radiated from a square centimeter of zirconia at the critical temperature as a function of ambient temperature. It shows more strikingly than does Figure 5 that at low furnace temperatures the safe radiation from a heater is very low, while with high temperatures the performance per square centimeter can be large. This indicates that a large radiating surface per unit of heat output is very desirable.

Thus critical temperature and safe radiation desiderata are determinable for the oxide resistor whose wall thickness should not be great enough to permit detrimental or excessive radial temperature gradients, and specific criteria are above

illustratively set forth for zirconia. No such radial gradients are present when, as has been assumed above for purposes of analysis, the assumed heating element is a solid cylindrical element so small in diameter and hence so small in cross section that its temperature is uniform throughout its cross section. Nor are they present in the large-bore thin-walled tube used in some of the above calculations. The latter, a large-bore thin-walled tubular heating element, is in effect an assembly

of small-cross-sectioned parallel elements equally and uniformly energized electrically, and the conditions for stability within that assembly so energized are the same as those described above. Moreover, the thin-walled tube used in these calculations also meets the criterion for wall thickness earlier above set forth; the wall thickness is not great enough to permit excessive radial temperature gradients. The conditions for stability apply equally well to the stability of a multiplicity of identical heating elements connected in parallel in a furnace. It has been

amply confirmed in experimental furnaces.

Accordingly, in operating furnaces constructed according to my invention, initial heating of the zirconia tube is effected as above described, as by using gas or a temporarily inserted resistance element, the zirconia tube being heated substantially uniformly to a temperature on the order of  $1400^{\circ}$  C., whereupon the tubular heating element is connected to the power supply and control circuit as above described. The zirconia heater tube meets the criterion of wall thickness above set forth, and the provisions above described insure that the current flows into and out of the tubular element at uniform current density throughout the above described contact faces or surfaces at the respective ends thereof, and this action is assured though the parts partake of temperature - responsive dimensional changes. The preliminary heating, as by gas or an inserted resistor, has made the heater tube sufficiently conductive for the flow of current from one end to the other and the current flows therethrough at substantially uniform density throughout any cross section taken between the ends of the heat-

## 11

er tube. It functions in effect like a set of small-cross-sectioned individual elements arranged integrally in a circle, and because the above relationship of wall thickness to inside diameter is not departed from, if any one of these imaginary elements or subdivisions of the zirconia tube heats up beyond the others, it can and does lose more heat by radiation than it gains, and thus the conditions that are otherwise conducive to channeling are counteracted. Thus continued heating up of the heater tube is facilitated, as is also subsequent operation of the furnace at the desired ultimate furnace temperature.

This action of continued heating up after the current is turned on will thus also be seen to contribute toward maintaining uniform current density, and thus uniform heating up is reliably and more quickly attained. The action just above described might be said to achieve substantially automatic maintenance of temperature equilibrium throughout the mass of the heater, and a similar substantially automatic action takes place during the run of the furnace at its ultimate furnace temperature at which treatment of articles or materials is desired to take place.

It is preferred to supply energy to the hollow cylindrical element of the furnace under conditions of constant current control, effected by setting the current regulator of the supply system of Fig. 7 to the desired current value, the regulator being manually set to function at the selected standard or value of current to be kept constant. It is possible, once the heater has been sufficiently heated by an extraneous source, to close the circuit and set the regulator at a current value that will ultimately give the desired operating furnace temperature upon completion of the heating up by the current itself, for the above-described dimensional criterion or characteristic of the zirconia tubular heater and the limitation of current or amperage effected by the current regulator coact to achieve prevention of conditions of instability such as those described above in connection with Figure 4. Because of such coactions and by setting the current regulator to successively different standards of operation, it is also possible to supply current to the heater tube at a different value during the heating-up period than is supplied during the continued operation of the furnace at its desired temperature, so long as the change in value is effected with due regard to the otherwise inherent conditions of stability and of instability that exist, respectively, to the left and to the right of the maximum points of the graphs, such as those of Figure 4, for the heater element. Because of the wide range of stability that exists to the left of the knee in the graphs, precision and closeness of control can be departed from and energization, throughout that range of stability, could even be effected at higher current values or at varying current values such as accompany the application of the electrical energy at constant voltage, and in this latter connection the energy could be applied in successive stages at successively different standards of constant voltage, if desired—provided, of course, as will now be clear, that substantial precision and closeness of constancy of current be instituted just before or when the critical temperature is reached, for thereafter, as above explained and demonstrated, conditions of instability can be brought about at potentials and temperatures to the right of the maximum point in the corresponding graph like that of Figure 4.

## 12

However, once the current is turned on after the preliminary heating by an extraneous source, it generally will be preferable to maintain constancy of current regulation at a single and appropriate current value which, for the particular tubular heater element, will insure continuity of conditions of stability throughout. In this preferred method, the further advantage is achieved in that the continued heating up that goes on

10 after the removal of the extraneous heat source takes place relatively slowly, which is desirable because it lessens any tendency toward non-uniform heating up throughout the cross section of the tubular element; the selected current value, of course, is one that is within the limits of the conditions for stability to the left of the maximum point or points in the graphs of Figure 4, and while, as earlier explained above, a voltage that is safe at a low furnace temperature may become excessive at higher temperatures, the voltage at which the selected current value is delivered to the heater unit after the ultimate furnace temperature is reached is, therefore, well within a safe value during the heating-up stage.

15 20 25 For example, for the furnace of Figure 2, an ultimate furnace temperature of 1600° C. may be desired and in that case, after preliminary heating to about 1400° C., the current is turned on with the regulator set to maintain current flow constant at 20 amperes. After turning on the current, so that the heating up proceeds at a constant current flow of 20 amperes, the voltage drops slowly to a value of about 127 volts and the furnace temperature levels off at 1600° C., giving 30 35 a power input of about 2540 watts. To illustrate the functioning of the intermediate and end blocks, the temperature of the intermediate block was about 1030° C. (measured at the bottom of a hole therein one inch deep), and the zinc oxide end block had a temperature of 985° C.

40 Thus it will be seen that, by my invention, many thoroughly practical advantages are successfully achieved. I have operated furnaces constructed in accordance with this invention, at temperatures between 1600° C. and 1800° C., over substantial periods of time and without any trouble or difficulty. The risks, damage, losses, and limitations imposed or caused by channeling can be successfully avoided and controlled stability achieved according to the principles of my invention. While, so far as concerns the resistor element or elements per se, I have described my invention in connection with the use of zirconia resistor elements, and more particularly stabilized zirconia heater elements, I have done so 45 because of the over-all superiority and many novel advantages that I am enabled thereby to achieve, but I do not wish to be limited thereto except as such limitation may be expressed in one or more of the claims. Many of the advantages and various of the results of my invention may be achieved by utilizing other known refractory oxides that are conducting at high enough temperatures. Of course, elements of expense or 50 55 60 65 cost of some of these will enter as a consideration in their practical application. Also, the particular characteristics of any one or more of such other refractory oxides might make it more suitable for some particular purpose; for example, for very high temperatures, thoria may be employed in preference to zirconia because, for example, it has a higher melting point. Whatever the selected refractory oxide, stability of operation may be achieved according to the principles fully explained and illustrated above in connection with

70 75

## 13

the use of stabilized zirconia, as for example, by shaping it in the form of a tube in which the relation between the inside diameter and wall thickness is such that detrimental or excessive radial temperature gradients are not produced, and supplying electrical energy thereto so controlled that ambient temperature and resistor temperature are maintained within those ratios that mean stability, as is illustratively explained above in connection with stabilized zirconia tubular resistors.

It will also be seen that some known disadvantages or limitations met with heretofore are overcome, according to my invention, by the use of zirconia tubes instead of solid rods, others by the use of stabilized zirconia, others by the use of intermediate cold ends and outer cold ends, all as illustratively above described. Nor do I wish to be limited, in the making of the outer cold ends, to the oxides I have above mentioned specifically, except as any such limitation is set forth in any of the claims; other known conductive refractory oxides are also usable in the making of these cold ends, so long as they have a suitable lower resistivity than that of the heater element and otherwise conform to the principles of my invention as illustratively described above in connection with these outer cold ends and their action with other parts.

It will thus be seen that there has been provided by this invention a high temperature resistor in which the various objects hereinabove set forth together with many thoroughly practical advantages are successfully achieved. As many possible embodiments may be made of the invention and as many changes might be made in the embodiment above set forth, it is to be understood that all matter hereinbefore set forth or shown in the accompanying drawings is to be interpreted as illustrative and not in a limiting sense.

I claim:

1. A high temperature electric furnace comprising means forming a refractory heat-resistant enclosure having therein a tubular heater element made of a refractory oxide that has a negative temperature coefficient of resistance, said tubular element being substantially non-channeling, having a substantially uniform cross section throughout its length and having a wall thickness less than that at which, throughout the desired operating temperatures, heat is generated internally of the refractory oxide at a rate greater than the rate at which said tubular element loses heat from its wall surface, and means 50 coaxing with its respective ends for engaging said tubular heater element for subjecting it to axial compression free from radial stresses on said ends and for supplying electrical energy to it in substantially uniform distribution thereto throughout the 360° extent at each end, comprising a succession in axial direction of contacting end blocks at each end face of said tubular heater element, said end blocks being relatively massive per unit length compared to the mass of said tubular element per unit length and each succession of end blocks comprising an inner current-distributing end block having a seat of 55 360° extent for making uniform surface engagement with and throughout the 360° extent of the 70 annular end face of the tubular heater element and made of a refractory oxide having substantially the same characteristics as that of said heater element and an outer end block made of a refractory oxide having a lower resistivity than 75

## 14

that of the oxide of the inner end block and making conductive contact with the latter throughout an area of contact of the latter with the tube end, substantial surface areas of said outer end blocks being exposed externally of said furnace enclosure for heat loss, and means for making electrical connections to said outer end blocks comprising metallic means of large exposed heat-radiating surface and interengaged with the outermost end block of said furnace enclosure of substantially uniform current distribution thereto.

2. An electric furnace as claimed in claim 1 in which the oxide of said tubular element is stabilized zirconia that comprises the reaction product under heat of zirconia with lime, of a quantity on the order of from about 3% to about 6% of the amount of zirconia.

3. An electric furnace as claimed in claim 1 in which the refractory oxide of said tubular element is selected from the group consisting of zirconia and thoria, stabilized, containing from 3% to 6% of alkaline oxide selected from the group consisting of lime and magnesia.

4. An electric furnace as claimed in claim 1 in which the inner block of each of said succession of contacting end blocks comprises a solid cylinder of said refractory oxide which is provided with an annular recess in an end of the solid cylinder to receive an end portion of said tubular element for making said uniform current-distributing surface engagement throughout the 360° extent of the contacting surfaces.

5. An electric furnace as claimed in claim 1 in which said inner block of each of said succession of contacting blocks comprises a ring-shaped member of substantial radial dimension compared to the thickness of the wall of said tubular member, said ring-shaped member having a 40 coaxial annular recess for receiving an end portion of said tubular element for making uniform current-distributing engagement throughout the said 360° extent of the contacting surfaces.

6. A high temperature electric furnace comprising a refractory heat-resistant enclosure and having therein a heater element made of a refractory oxide that has a negative temperature coefficient of resistance and that is substantially non-channeling, having a ratio of external surface to cross sectional area greater than that at which, for any operating temperature, heat is generated internally thereof at a rate faster than said element can lose heat through its surface, a constant current source of electrical energy having means connecting it to supply current to the respective ends of said oxide heater element substantially uniformly distributed throughout the 360° extent thereof, and means for manually setting the value at which current supplied to said heater element is kept constant whereby said oxide heater element may be heated up at a low rate within its voltage factors of stability for the respective successive heating-up temperatures and may be thereafter supplied at a relatively high value of constant current at relatively low voltage within its voltage factors of stability for the temperature of continued furnace operation.

7. The steps in a method of preventing channeling in a high temperature electric furnace resistor element that is made of a refractory oxide that has a negative temperature coefficient of resistance which comprise providing the oxide resistor element with a surface area greater than that at which heat is generated therein at a greater rate than, for any given temperature, is

lost by the element through its surface, heating the oxide resistor element substantially uniformly by means of an extraneous source of heat until it becomes significantly conductive, then supplying electrical energy thereto uniformly distributed to it at its respective ends and throughout the 360° extent of the latter and at a relatively low rate to slowly heat it up to operating temperature and in so doing maintaining the applied voltage of the current within the voltage factors of stability of the oxide resistor element for the respective successive heating-up temperatures, and thereafter supplying the oxide resistor element with current at relatively high amperage and at relatively low voltage within the voltage factors of stability of the oxide resistor element for the temperature of continued furnace operation.

8. A high temperature resistor unit for electric furnaces comprising a heater element in the form of a hollow cylinder made of a refractory oxide that has a negative temperature coefficient of resistance with means for making electrically conductive contact with at least one end of said cylinder, said means comprising a member of materially greater cross section than that of said hollow cylinder and made of a refractory oxide of substantially the same negative temperature coefficient of resistance as that of said hollow cylinder and having a face for surface contact with an annular face of said hollow cylinder whereby pressure of surface contact therebetween places said refractory cylinder under stress in axial direction and said refractory cylinder is free of stressing in radial direction, and a member in surface engagement with said first-mentioned member and made of a material which has a lower resistivity than that of said first member and that is selected from the group consisting of zinc oxide, titanium oxide, magnetic iron oxide, copper oxide, manganese oxide, and uranium oxide.

9. A resistor unit comprising a tubular element made of a refractory oxide that has a negative temperature coefficient of resistance, said tubular element being of substantially uniform cross section throughout its effective length and having a wall thickness not greater than that at which, throughout the desired operating temperatures and in response to electric current flow therein, heat is generated internally of the refractory oxide forming the wall of said tubular element at a rate greater than the rate at which said tubular element loses heat from its wall surface, thereby to resist channeling, and a "cold" end element abutting against the annular end face of said refractory oxide tubular element and made of a similar refractory oxide and of materially greater cross section than that of said tubular element and having a seat providing a surface of 360° extent for making surface contact with a surface of 360° extent at an end of said hollow cylinder for substantially uniformly distributing current to said end.

10. A resistor unit as claimed in claim 9 in which said "cold" end element comprises a solid cylinder of said refractory oxide and said seat comprises an annular recess in an end of said solid cylinder to receive an end portion of said hollow cylinder.

11. A resistor unit as claimed in claim 9 in which said "cold" end element comprises a ring-shaped member of substantial radial dimension compared to the thickness of the wall of said hollow cylinder and said seat comprises a sub-

stantially coaxial annular recess for receiving an end portion of said hollow cylinder.

12. A high temperature resistor for an electric furnace comprising a tubular element of refractory oxide selected from the group consisting of zirconia and thoria, stabilized, containing from 3% to 6% of alkaline oxide selected from the group consisting of lime and magnesia, said tubular element being of substantially uniform cross section throughout its effective length and having a wall thickness not greater than that at which, throughout the desired operating temperatures and in response to current flow therein, heat is generated internally of the wall mass of said stabilized refractory oxide at a rate greater than the rate at which said tubular element loses heat from its wall surface, thereby to resist channeling.

13. A high temperature resistor for an electric furnace comprising a tubular element of stabilized zirconia comprising the reaction product under heat of zirconia with lime of a quantity on the order of from about 3% to about 6% of the amount of zirconia, said tubular element being of substantially uniform cross section throughout its effective length and having a wall thickness not greater than that at which, throughout the desired operating temperatures and in response to current flow therein, heat is generated internally of the wall mass of stabilized zirconia at a rate greater than the rate at which said tubular element loses heat from its wall surface, thereby to resist channeling.

14. A high temperature resistor for an electric furnace comprising a tubular element of stabilized zirconia comprising the reaction product under heat of zirconia with an oxide selected from the group consisting of magnesia and lime of a quantity on the order of from about 3% to about 6% of the amount of zirconia, said tubular element being of substantially uniform cross section throughout its effective length and having a wall thickness not greater than that at which, throughout the desired operating temperatures and in response to current flow therein, heat is generated internally of the wall mass of stabilized zirconia at a rate greater than the rate at which said tubular element loses heat from its wall surface, thereby to resist channeling.

#### References Cited in the file of this patent

#### UNITED STATES PATENTS

| Number    | Name           | Date          |
|-----------|----------------|---------------|
| 684,296   | Nernst et al.  | Oct. 8, 1901  |
| 775,664   | Higgins        | Nov. 22, 1904 |
| 847,003   | Von Ischewsky  | Mar. 12, 1907 |
| 1,132,684 | Queneau        | Mar. 23, 1915 |
| 1,218,058 | Cope           | Mar. 6, 1917  |
| 1,308,878 | Thomson        | July 8, 1919  |
| 1,352,387 | Saunders       | Sept. 7, 1920 |
| 1,438,936 | Eimer          | Dec. 12, 1922 |
| 1,470,195 | De Roiboul     | Oct. 9, 1923  |
| 1,576,621 | Anderson       | Mar. 16, 1926 |
| 1,613,877 | Dyckerhoff     | Jan. 11, 1927 |
| 1,969,132 | Heyroth        | Aug. 7, 1934  |
| 2,231,723 | Jung et al.    | Feb. 11, 1941 |
| 2,268,691 | Brooke         | Jan. 6, 1942  |
| 2,294,034 | Jaeger         | Aug. 25, 1942 |
| 2,320,172 | Brooke et al.  | May 25, 1943  |
| 2,323,051 | Junker et al.  | June 29, 1943 |
| 2,404,060 | Hall et al.    | July 16, 1946 |
| 2,516,570 | Hartwig et al. | July 25, 1950 |